

## UNITED STATES PATENT OFFICE

2,036,161

## PRODUCING SYNTHETIC TANNING AGENTS

Hermann Schuette, Mannheim, Germany, assignor to I. G. Farbenindustrie Aktiengesellschaft, Frankfort-on-the-Main, Germany

No Drawing. Application July 27, 1934, Serial No. 737,260. In Germany August 8, 1933

15 Claims. (Cl. 149—5)

The present invention relates to synthetic tanning agents and a process of producing same.

I have found that valuable tanning agents can be obtained in a simple manner by causing a dihydroxydiphenylsulphone to react with a water-soluble salt of sulphurous acid and a formaldehyde substance (which expression means formaldehyde itself and substances supplying formaldehyde). The reaction is carried out at temperatures above 100° C. by heating under pressure, for example, by heating the reagents together with water in a closed vessel. Very suitable are temperatures between 100° and 200° C., for example from 140° to 160° C. As initial materials for the process according to this invention there may be mentioned, for example, 4,4'-dihydroxydiphenylsulphone, 4,4'-dihydroxy-3,3'-dimethyldiphenylsulphone, 2,2'-dihydroxydiphenylsulphone and also sulphones containing substituents, such as, for example, halogen atoms. The salts of sulphurous acid, for example, sodium, potassium or ammonium sulphite, and formaldehyde or trioxymethylene may be added to the said diphenylsulphones in aqueous solution. It is preferable to work at temperatures above 100° C. and while employing pressure, for example, by operating in a closed vessel. The amounts of formaldehyde and sulphurous acid salts to be employed are advantageously so selected that one or two  $-\text{CH}_2-\text{SO}_3\text{H}$  groups enter into the molecule of the sulphone. Any intermediate amounts may also be employed. If only the amount of formaldehyde be increased, a condensation of the sulphones with each other takes place.

The condensation products prepared according to this invention yield, after tanning, a leather which is distinguished by its fastness to light and which entirely fulfills the requirements of the modern leather industry. They are especially suitable for the manufacture of leather fast to light for uppers, portfolios and furniture, and for tanning reptile leathers in which it is desired to retain especially well the fineness of the design and the shade of colour. The said tanning agents frequently have a very good fulfilling action. They may be advantageously employed together with other natural or vegetable tanning agents, such as, for example, sumach or gall nut extract, or together with other synthetic tanning agents, for instance, those described in the copending application Ser. No. 727,913 or in Patent No. 1,336,759 and in Patent No. 1,237,405; furthermore they influence very favorably the

colour of the leather obtained by mineral (chrome) tanning.

The tanning agents obtainable according to the present invention, when in the form of a 1 per cent aqueous solution, yield, by the addition of a dilute aqueous solution of iron chloride, a reddish violet colouration which soon becomes turbid by the deposition of a reddish violet precipitate.

The following examples will further illustrate the nature of this invention, but the invention is not restricted to these examples. The parts are by weight.

## Example 1

125 parts of 4,4'-dihydroxydiphenylsulphone are introduced into a solution of 126 parts of calcined sodium sulphite and 150 parts of 30 per cent aqueous formaldehyde in 500 parts of water, the whole being heated for 36 hours at from 155° to 160° C. in a closed vessel. A yellowish-brown, clear solution is obtained; it is rendered acid to congo by means of a little, from 20 to 25 per cent aqueous sulphuric acid, boiled for a short time and filtered if necessary. The solution is then evaporated on a waterbath until it has a syrupy consistency or at room temperature in vacuo to dryness until a pale yellowish mass is obtained. A tanning agent is thus obtained which is especially suitable for tanning reptile leather.

## Example 2

125 parts of 4,4'-dihydroxydiphenylsulphone are introduced into a solution of 75 parts of calcined sodium sulphite, and 100 parts of 30 per cent aqueous formaldehyde in 300 parts of water; the whole is then heated for 4 hours at 150° C. in an autoclave. An aqueous solution is obtained which is diluted with about the same weight of water and then rendered acid to congo with dilute aqueous sulphuric acid of from about 20 to 25 per cent strength. The solution is then boiled for a short time, filtered if necessary and evaporated on a waterbath to give a viscous mass or in vacuo to dryness to give a dry, pale yellowish mass.

By the addition of concentrated hydrochloric acid to the aqueous solution, the reaction product may also be precipitated in the form of a colourless mass which may be separated after sedimentation and then freed from any hydrochloric acid and water still present by allowing it to stand over caustic soda at room temperature in vacuo.

30

35

40

45

50

55

55



ter in a closed vessel to a temperature between 140° and 160° C.

10. Tanning agents originating from the reaction of a dihydroxydiphenylsulphone, a water-soluble salt of sulphurous acid and a formaldehyde substance.

11. Tanning agents originating from the reaction of a dihydroxydiphenylsulphone, a water-soluble salt of sulphurous acid and formaldehyde.

10 12. Tanning agents originating from the reaction of 4,4'-dihydroxydiphenylsulphone, a water-soluble salt of sulphurous acid and formaldehyde.

13. Tanning agents originating from the reaction of 1 molecular proportion of 4,4'-dihydroxy-

diphenylsulphone, 1 molecular proportion of a water-soluble salt of sulphurous acid and 1.2 molecular proportions of formaldehyde.

14. Tanning agents originating from the reaction of 1 molecular proportion of 4,4'-dihydroxy- 5 diphenylsulphone, 1.2 molecular proportions of a water-soluble salt of sulphurous acid and 2 molecular proportions of formaldehyde.

15. Tanning agents originating from the reaction of 1 molecular proportion of 4,4'-dihydroxy- 10 diphenylsulphone, 2 molecular proportions of a water-soluble salt of sulphurous acid and 2 molecular proportions of formaldehyde.

HERMANN SCHUETTE.